

## UNITED STATES PATENT OFFICE

2,226,335

## LUBRICATING OIL COMPOSITION, CONSTITUENT THEREOF, AND METHOD OF MANUFACTURING THE SAME

Troy Lee Cantrell and James Otho Turner, Lansdowne, Pa., assignors to Gulf Oil Corporation, Pittsburgh, Pa., a corporation of Pennsylvania

No Drawing. Application September 14, 1936, Serial No. 100,786

8 Claims. (Cl. 252—53)

Our invention relates to lubricating oils and in particular to lubricating oil compositions containing an oil-soluble agent or agents effective to impart so-called "extreme-pressure" characteristics thereto, and also having certain additional advantages as set forth hereinbelow.

Despite the many technical advances which have been made in the arts of refining and applying lubricating oils, modern lubricating oils and bearings often fail to perform satisfactorily. It is well known in the art that straight petroleum lubricants have fairly well defined limits of bearing speeds, pressures and temperatures, within which they will give acceptable service. These limitations are often reached and even exceeded in modern engines, gears and the like, resulting in machines that cannot be satisfactorily lubricated by straight mineral oils. Such modern designs have been brought about through constant attempts on the part of engineers to improve engines and machines with respect to compactness, speed, power and acceleration. In order to provide satisfactory lubrication for modern designs and keep pace with new mechanical improvements in design, it is necessary to provide lubricating compositions having improved lubricating value as compared with straight lubricating oils and which will give satisfactory service under drastic lubricating conditions under which straight mineral oils would fail to perform satisfactorily.

Thus, considerable attention is being paid to the development of lubricating oil compositions which are capable of giving satisfactory service under high pressures, such compositions being generally known in the art as "extreme-pressure" or "EP" lubricants. A number of materials have been developed which, when added to hydrocarbon oil, materially increase the extreme-pressure properties of the oil; the resultant compositions give more acceptable service under higher pressures between bearing surfaces than is true of the untreated oil. Some of these agents are extremely effective but too expensive for general use, and others, while contributing satisfactory extreme-pressure properties to the oil, are unsatisfactory for other reasons. A primary requisite of any improvement agent is good oil-solubility under service and marketing conditions; such agents when added to hydrocarbon oils in small amounts should not impart to the resulting composition a hazy or cloudy appearance, should not deposit out when the compositions are stored and packaged prior to sale, and should not attack metal surfaces of containers after being

packaged and stored. The improvement agent should also be highly effective per unit concentration in the lubricating oil compositions; otherwise it would be necessary to add such an amount of the improvement agent as to substantially modify many of the desirable physical properties of the lubricating oil itself. Such oils have been carefully refined to meet exacting specifications, and if it is necessary to incorporate therein relatively large amounts of some agent or agents differing in physical properties from the oil itself, the resulting compositions may prove unsatisfactory for the purposes for which the lubricating oils were prepared. In general it is desirable that any improvement agent should be effective at concentrations not exceeding 1 or 2 per cent, or at the most 5 per cent, by weight of the lubricating oil.

For many purposes it is not necessary to increase the load-carrying properties of lubricating oils to several times the load-carrying properties of the original oils. For example, in the lubrication of automotive engines, difficulty is frequently encountered at points where the pressures between bearing surfaces are not extremely high. Difficulties are thus frequently encountered in maintaining effective lubrication between piston rings and the side walls of the cylinders, due to the fact that the temperatures of the surfaces may run very high. With ordinary mineral lubricating oils it may be impossible or difficult to provide safe and effective lubrication for mechanically efficient engines having a tendency to develop high temperatures at this point. While this difficulty is due primarily to temperature, it has been found that lubricating oils containing small amounts of extreme-pressure agents give better results under these conditions; these results have been variously explained but are probably due to the fact that such extreme-pressure agents wet or adhere to the metal and the oil wets or adheres to the extreme pressure agent.

It is, therefore, an object of our invention to provide an improvement agent or agents of the character indicated herein, having the property of imparting desirable extreme-pressure characteristics to hydrocarbon oils when incorporated therein, which agent or agents shall be free from many or all of the disadvantages of agents previously employed for the same general purpose, as well as inexpensive to produce.

A further object of our invention is to provide improved lubricating compositions comprising

carrying the absorption of olefin farther is to make the anti-oxidant product less capable of absorbing the desired amount of phosphorus in the final stage.

- 5 When the anti-oxidant starting material is prepared from phenol ( $C_6H_5OH$ ) itself, e. g. "90 per cent phenol," the degree of absorption of olefin may be carried farther, for example to about two mols of olefin per mol of phenol (based on the assumption that the olefin is made up entirely of  $C_4$  hydrocarbons).

- 10 The preferred olefins are those containing from three to eight carbon atoms per molecule; the higher the molecular weight of the olefin, the more viscous the final phosphorus-containing product will be. Olefins containing more than eight carbon atoms per molecule tend to reduce the phosphorus content of the final inhibitor product. Ethylene ( $C_2H_4$ ), on the other hand, is insufficiently reactive, requiring the use of fuming sulfuric acid and does not sufficiently reduce the acidity of the original phenol.

latter being a recovered acid obtained from acid sludge produced in washing hydrocarbon oil with sulfuric acid. The 90 per cent phenol employed had the following properties:—

|                                             |       |   |
|---------------------------------------------|-------|---|
| Specific gravity: $60^{\circ}/60^{\circ} F$ | 1.050 | 5 |
| Melting point, capillary tube: $^{\circ}F$  | 91.9  |   |
| Color: NPA                                  |       | 5 |

15 The phenol was placed in a suitable iron vessel and heated to a temperature of  $120^{\circ} F$ . Olefinic gas was then introduced slowly to agitate the phenol and the acid was added in two batches, 10 lb. at first and the remaining 10 lb. two hours later. The temperature at the end of two hours was  $150^{\circ} F$ ., and the mixture was maintained at 15 this temperature for 16 hours, olefinic gas being passed through the mixture during this time at the rate of 1600 cu. ft. per hour. The operation was conducted under a pressure of from 15 to 25 lb. per sq. in.

20 The olefinic gas employed in this example was

25 The best olefin starting materials are those containing from three to eight carbon atoms per molecule. From gases produced in the cracking of hydrocarbons, fractions obtained

30 specific gravity of 1.00 and having a

5 mains that anti-oxidants may be prepared in the manner set forth hereinbefore and in the aforesaid co-pending applications, and such materials comprise suitable starting materials for  
 10 5 the manufacture of phosphorus-containing improvement agents in accordance with our present invention; certain of the constituents of the anti-oxidant starting materials which are not in themselves effective as anti-oxidants may, nevertheless, be capable of being converted by reaction with phosphorus oxychloride to materials having useful properties for the purposes in view.

15 We prefer to employ as starting materials anti-oxidants, prepared as set forth above and in the aforesaid co-pending applications, having physical properties within the following range:

|                                      |                        |
|--------------------------------------|------------------------|
| 20 Gravity: °API                     | 15.0 to 25.0           |
| Specific gravity:                    |                        |
| 60°/60° F.                           | 0.9659 to 0.9042       |
| Viscosity, S.U.V at 100° F.: seconds | 150 to (solid)         |
| 25 Color:                            | Water white to 7 (NPA) |
| Pour point (liquids only): °F.       | 0 to 30                |
| Melting point (solids only): °F.     | 80 to 225              |

30 Our invention in its broadest aspects, however, is not limited to the preferred starting material mentioned hereinabove but contemplates the manufacture of inhibitors of the general class described from any alkylated phenols so long as such alkylated phenols possess definite anti-oxidant properties, are insoluble in water, insoluble or only slightly soluble in dilute alkali, and are permanently soluble up to 5 per cent in 35 paraffin oils. For example, we may employ as starting materials anti-oxidants prepared by reacting various light cracked hydrocarbon distillates and other normally liquid olefinic hydrocarbon mixtures with phenol, in the presence of 40 sulfuric acid, as described in the aforesaid co-pending applications. It is a requisite of such olefin-phenol reaction products, however, insofar as the present process is concerned, that one or more secondary and/or tertiary carbon linkages be present in the compound.

45 The anti-oxidant value of this starting material should be such that the addition of 0.01 per cent by weight thereof to standard gasoline stock having an oxygen stability test (E. G. C. Method) 50 of, say, 120 minutes, will raise the oxygen stability test to at least 240 minutes. Less potent anti-oxidants are unsuitable as starting materials.

55 As aforesaid, we prepare our present improvement agents by reacting anti-oxidants of the general character described hereinabove with phosphorus oxychloride. The reaction is conducted by mixing phosphorus oxychloride with 60 the anti-oxidant material in the desired amount and heating the mixture until the latter is substantially free from chlorine or chlorides, temperatures of around 300° or 400° F. being suitable for this purpose.

65 70 In general we have found it advantageous to limit the amount of phosphorus oxychloride added so as to yield a product containing from about 1 to 5 per cent of phosphorus, assuming the anti-oxidant starting material to be free or 75 relatively free from diluents; if the phosphorus

content substantially exceeds 5 per cent, the resulting product tends to be insufficiently soluble in lubricating oils, especially highly paraffinic lubricating oils. Also, in such case, the product tends to be too active at temperatures below, say, 250° F. By limiting the addition of phosphorus oxychloride to such an extent as will leave some of the original anti-oxidant material unaltered, for example by adding a sufficient amount of phosphorus oxychloride to a concentrated anti-oxidant to yield a product containing around 1 to 3 per cent of phosphorus, it is possible to obtain products which possess desirable extreme-pressure characteristics while at the same time retaining to a considerable extent the anti-oxidant and stabilizing properties of the original starting material. Moreover, the unreacted anti-oxidant serves as a blending agent for the relatively less soluble phosphorus oxychloride reaction product.

20 Before being brought into contact with phosphorus oxychloride, the anti-oxidant material should be dried to remove any substantial amount of moisture contained therein. Phosphorus oxychloride is then slowly added to the desired anti-oxidant, the mixture being vigorously agitated by suitable mechanical means during the addition. During the addition period there is a copious evolution of hydrogen chloride, and for this reason it is well to add the phosphorus oxychloride well below the surface of the liquid to avoid being swept out by the evolved gas and lost. When the desired amount of phosphorus oxychloride has been added, the temperature is slowly raised to around 300° to 400° F., and the mixture is maintained at this elevated temperature until there is no further evidence of hydrogen chloride evolution, and preferably until the hydrogen chloride content of the product is less than 0.30 per cent. The resultant product, after 30 cooling, represents the finished improvement agent of our invention and as such is ready for addition to lubricating oils without further purification.

45 The character of the final phosphorus-containing inhibitor will, of course, vary with the character of the phenolic and olefinic material employed in the manufacture of the anti-oxidant starting material, with the extent of absorption of the olefin, and with the amount of phosphorus 50 subsequently introduced. All of these factors are, however, very intimately interrelated. These are the primary factors, but it will be obvious that there are numerous secondary factors, for example the degree of purification and decolorization of the anti-oxidant starting material.

55 Naturally, it is to be expected that the viscosities, specific gravities and other physical characteristics of the particular phenols employed have a corresponding effect upon the product, to some extent at least; this effect may, however, not always hold true where the degree of olefin absorption varies over comparatively wide limits and where the percentage of phosphorus in the 60 final compound also varies.

65 When cresylic acid, ortho-cresol and meta-cresol and the like are used in the manufacture of the anti-oxidant, we prefer to limit the olefin absorption to around one mol per mol of the phenolic material, i. e. to give a water-insoluble product representing roughly 135 to 150 per cent by volume of the original phenol, in order ultimately to secure inhibitors that are sufficiently soluble in the higher gravity oils; the result of 70 75

carrying the absorption of olefin farther is to make the anti-oxidant product less capable of absorbing the desired amount of phosphorus in the final stage.

5 When the anti-oxidant starting material is prepared from phenol ( $C_6H_5OH$ ) itself, e. g. "90 per cent phenol," the degree of absorption of olefin may be carried farther, for example to about two mols of olefin per mol of phenol (based on the assumption that the olefin is made up entirely of  $C_4$  hydrocarbons).

10 The preferred olefins are those containing from three to eight carbon atoms per molecule; the higher the molecular weight of the olefin, the more viscous the final phosphorus-containing product will be. Olefins containing more than eight carbon atoms per molecule tend to reduce the phosphorus content of the final inhibitor product. Ethylene ( $C_2H_4$ ), on the other hand, is insufficiently reactive, requiring the use of fuming sulfuric acid and does not sufficiently reduce the acidity of the original phenol.

15 The best olefin starting materials are those containing from three to five carbon atoms per molecule, especially butylenes; fractions obtained from gases produced in the pyrolysis of hydrocarbon oils and rich in olefins of this approximate range represent advantageous and available raw materials.

20 30 After the reaction between the phenol and olefin has been carried to the desired degree of completion, the product is washed with water and dilute caustic soda in the manner set forth hereinabove and in the aforesaid co-pending applications. The resultant water-insoluble anti-oxidant material is then preferably dried. The drying may be accomplished by filtering this material through adsorbent clay or the like, the effect of which is to dehydrate and decolorize. Or, the 35 drying may be accomplished by heating the anti-oxidant material to about 400° F. in suitable apparatus; this procedure dehydrates and tends to darken the anti-oxidant material.

40 45 The dry anti-oxidant may then be treated directly with the phosphorus reagent, or it may first be distilled to separate undesirable low-boiling and high-boiling constituents, respectively. Thus we may distill under a vacuum of from -11 inches to -28 inches of mercury, recovering a 50 fraction distilling over between 300° and 550° F., which fraction may then be treated with phosphorus oxychloride. The lower boiling material, and sometimes also the residue, may be recycled 55 for further reaction with olefins in the presence of sulfuric acid, or used as an anti-oxidant.

55 60 It is, in fact, ordinarily desirable to employ such distillation, or to filter the anti-oxidant, and sometimes even a distillate fraction thereof through a solid adsorbent material such as fuller's earth or the like, in order to lighten the color of the starting material prior to treatment with phosphorus oxychloride, inasmuch as the latter treatment tends to have a darkening effect. 65 It will be understood that a light color is a desirable characteristic with respect to any improvement agent intended to be added to mineral oils.

70 The following example will serve to illustrate our invention:

#### EXAMPLE 1

##### (a) Preparation of anti-oxidant starting material

75 50 gallons of "90 per cent phenol" were mixed with 20 pounds of 98 per cent "black acid," the

latter being a recovered acid obtained from acid sludge produced in washing hydrocarbon oil with sulfuric acid. The 90 per cent phenol employed had the following properties:—

|                                |            |       |   |
|--------------------------------|------------|-------|---|
| Specific gravity:              | 60°/60° F. | 1.050 | 5 |
| Melting point, capillary tube: | °F.        | 91.9  |   |
| Color:                         | NPA        |       | 5 |

10 The phenol was placed in a suitable iron vessel and heated to a temperature of 120° F. Olefinic gas was then introduced slowly to agitate the phenol and the acid was added in two batches, 10 lb. at first and the remaining 10 lb. two hours later. The temperature at the end of two hours was 150° F., and the mixture was maintained at 15 this temperature for 16 hours, olefinic gas being passed through the mixture during this time at 20 the rate of 1600 cu. ft. per hour. The operation was conducted under a pressure of from 15 to 25 lb. per sq. in.

25 The olefinic gas employed in this example was a cracked hydrocarbon gas fraction obtained in the pyrolysis of hydrocarbon oil, and having a specific gravity of 1.785. Upon agitation of a sample of this gas with 64 per cent sulfuric acid, 25 the acid absorbed 12.5 per cent by volume of the gas, which may be considered as isobutylene and dienes. The remainder of the sample lost 20 per cent by volume (based on the original volume of gas) by absorption in 87 per cent acid, which may 30 be considered as propylenes, butylenes and similar constituents. The remainder of the sample, upon being washed with bromine water, following the two acid washes, lost 2.6 per cent by volume (based on the original volume of gas), which 35 may be considered as ethylene. The gas, therefore, contained 34.1 per cent by volume of unsaturated constituents.

40 Upon completion of the operation, there was produced a material representing 300 per cent by volume of the original phenol, i. e. 150 gallons.

45 The crude product was then raised from 200° to 212° F., and 20 gal. of 10 per cent caustic soda solution were added to neutralize the sulfuric acid present. The resultant product, after removal of the caustic layer, was washed with boiling water, live steam being introduced during the washing operation, and was then allowed to settle for two hours after which the aqueous layer 50 was withdrawn. The remaining material was blown with air for two hours in order to reduce the moisture content of the product to two per cent by weight.

55 The final product, produced as set forth hereinabove, had a volume of 135 gallons and comprised a mixture of about 90 per cent of an oil-soluble material having anti-oxidant properties, and about 10 per cent of what appear to be gasoline-like polymers. It is a highly satisfactory 60 anti-oxidant and gum-inhibitor. Typical physical properties of products as thus prepared are as follows:

|                            |         |      |    |
|----------------------------|---------|------|----|
| Gravity:                   | °API    | 21.6 | 65 |
| Viscosity, SUV at 100° F.: | seconds | 122  |    |
| Color:                     | NPA     | Dark |    |
| Pour point:                | °F.     | 0    |    |

70 An anti-oxidant material prepared as set forth hereinabove was then distilled under a moderate vacuum, the distillate being cut into three fractions. That fraction distilling over at vapor temperatures between 400° and 550° F. was segregated for treatment with phosphorus oxychloride 75

as described below. Typical properties of fractions prepared in this manner are as follows:

|                         |      |
|-------------------------|------|
| Gravity: °API           | 18.6 |
| Viscosity, SUV: seconds |      |
| @ 100° F                | 211  |
| @ 210° F                | 36.4 |
| Pour point: °F          | -5   |
| Color: NPA              | 2.0  |

10 (b) *Preparation of final improvement agent*

15 80 parts by weight of a fraction prepared as set forth hereinabove were treated with 20 parts by weight of phosphorus oxychloride, the product being that described in an earlier portion of this specification. The resulting material had the following properties:

|                                  |              |
|----------------------------------|--------------|
| Gravity: °API                    | 51           |
| Viscosity, SUV: seconds @ 100° F | 1176         |
| Pour point: °F                   | 0            |
| Color, NPA                       | 5.5 (dilute) |
| Phosphorus: % by wt              | 3.98         |

20 The improvement agents prepared in accordance with our invention, and as exemplified by that given in the foregoing example, are all excellent improvement agents for addition to hydrocarbon lubricating oils and when added thereto in amounts up to 1 or 2 per cent by weight result in improved and advantageous lubricating compositions having desirable extreme-pressure characteristics.

25 These agents are permanently soluble in hydrocarbon oils, even in highly paraffinic oils, and are stable at ordinary temperatures. When added to lubricating oils in the amounts noted, they do not tend to settle out nor form sludge or deposition nor attack metal surfaces such as those of tin plate, terne plate, bronze or the like when packaged and stored prior to sale and use, or under circumstances of actual use in which the temperatures do not exceed, say, 250° F. On the other hand they are effective to contribute extreme-pressure properties to hydrocarbon oils even at atmospheric temperatures.

30 40 45 Not only do these materials have excellent extreme-pressure properties, but their chemical nature is such that should any hydrolysis occur, the organic products of such hydrolysis are in themselves anti-oxidant materials; in this respect our products differ sharply from simple aryl esters of phosphorus acids, such as triphenyl phosphite, which upon hydrolysis yields highly corrosive phenol.

50 55 60 65 In our process the phosphorus content of the final product may be varied by adjusting any one or more of the following factors: (1) the character and molecular weight of the phenolic starting material, (2) the character and molecular weight of the olefinic starting material, (3) the degree of olefin absorption in the phenolic reaction mixture, and (4) the relative amount of phosphorus oxychloride added to the phenol-olefin reaction product or anti-oxidant material. All of the above factors also exert a definite influence upon the color, solubility and viscosity of the final product. The color and concentration of the anti-oxidant material have a special influence upon the color of the ultimate improvement agent.

70 75 80 We, therefore, regulate these various factors with reference to each other and with regard to the starting materials available, in order to secure products of desired temperature-responsiveness, activity, solubility, viscosity, color and extreme-pressure action, within limits corre-

sponding to the use to which the final compositions are to be subjected. It will also be clear that we may limit the amount of the improvement agent added to any given hydrocarbon oil, to the same end.

85 90 95 100 105 110 115 120 125 130 135 140 145 150 Wherever the expression "highly paraffinic oil" is employed herein it is intended to indicate lubricating oils conforming in physical properties to oils prepared from Pennsylvania crudes; these "highly paraffinic oils" are either oils derived from Pennsylvania crudes, or oils which have been refined or blended to approach or even exceed the latter oils in paraffinity. Where various materials are referred to as being soluble in such paraffinic oils, this expression is intended to mean that such materials may be incorporated into such oils in the amounts required, without producing any haziness or cloudiness in the appearance of the resultant compositions, at least under atmospheric temperatures and under the ordinary conditions to which such oil compositions are subjected in storage and handling prior to their actual use as lubricants.

155 160 165 170 175 180 185 190 195 200 205 210 215 220 225 230 An advantage of our process and products is that the principal ingredients employed in the manufacture of the final products, namely olefins, are cheap and available to the refiner.

230 235 240 245 250 255 260 265 270 275 280 285 290 295 300 The following table will serve to illustrate the effectiveness of our improvement agents and the value of lubricating compositions containing them:

TABLE I

|                               | Untreated oil | Oil with addition of improvement agent as prepared in Example 1 | 35 |
|-------------------------------|---------------|-----------------------------------------------------------------|----|
| Make-up: Percent by wt.:      |               |                                                                 | 40 |
| Lubricating oil, SAE 10 grade | 100           | 99                                                              |    |
| Improvement agent             |               | 1.0                                                             |    |
| General properties:           |               |                                                                 |    |
| Gravity: °API                 | 27.8          | 27.2                                                            |    |
| Specific gravity: 60°/60° F   | 0.8883        | 0.8916                                                          |    |
| Viscosity, SUV: seconds.      |               |                                                                 |    |
| 100° F                        | 345           | 349                                                             |    |
| 130° F                        | 160           | 162                                                             | 45 |
| 210° F                        | 54.1          | 55.1                                                            |    |
| Viscosity index               | 92            | 96                                                              |    |
| V-G constant                  | 0.827         | 0.832                                                           |    |
| Flash, OC: °F                 | 425           | 420                                                             |    |
| Fire, OC: °F                  | 495           | 495                                                             |    |
| Pour point: °F                | 0             | +5                                                              |    |
| Carbon residue: percent       | 0.15          | 0.16                                                            | 50 |
| Phosphorus: percent by wt     |               | 0.04                                                            |    |
| Appearance                    | Clear         | Clear                                                           |    |
| Almen test:                   |               |                                                                 |    |
| Journal speed: RPM            | 600           | 600                                                             |    |
| Rubbing speed: ft. per min    | 40            | 40                                                              |    |
| Lever load: lb.               | 8             | 16                                                              |    |
| Torque: lb. ft. × 10          | 13            | 23                                                              |    |
| Unit load: lb./sq. in.        | 4000          | 8000                                                            | 55 |
| Lubricant temperature: °F:    |               |                                                                 |    |
| Initial                       | 86            | 86                                                              |    |
| Final                         | 113           | 114                                                             |    |

60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 Various modifications in the operating procedures mentioned hereinabove will suggest themselves to those skilled in the art. For example, we have described washing the phenol-olefin reaction product with water and dilute caustic soda solution to effect neutralization and removal of the acid or acids (e. g. sulfuric acid and sulfonic acids) remaining in the reaction mixture after the introduction of the olefins has been discontinued. Such neutralization and removal may be effected in other ways, as by extraction with aqueous alcohol, contact with solid alkalis such as lime or sodium carbonate, or by contacting the reaction mixture with solid adsorbents such as fuller's earth, activated carbon, or the like.

While our improvement agents, prepared as described hereinabove, may be added to hydrocarbon oils without admixture of other substances, advantageous results may be obtained by adding these improvement agents in conjunction with other agents and particularly agents having anti-oxidant and corrosion-inhibiting properties. Especially effective composite improvement agents may be prepared by using mixtures of our improved extreme-pressure agents, described hereinabove, with inhibitors prepared by treating anti-oxidant starting materials similar to those set forth hereinabove with phosphorus trichloride, as set forth in our co-pending application, Serial No. 99,662, filed September 5, 1936, or with phosphorus pentasulfide or a mixture of phosphorus pentasulfide and phosphorus trichloride, as set forth in our co-pending application, Serial No. 100,382, filed September 11, 1936. These composite mixtures may be prepared by treating the anti-oxidant starting material with mixtures of these phosphorus-containing reagents; for example, we may use as a reagent a mixture of phosphorus oxychloride and phosphorus trichloride. In all cases, the ultimate products should not contain more than about 5 per cent by weight of phosphorus. We have found that the results obtainable while using such composite mixtures in many cases exceed the sums of the results obtained by using the individual improvement agents alone. Thus, the materials described in the co-pending applications referred to in this paragraph are found to exert a certain stabilizing effect upon the action of the extreme-pressure agents prepared in accordance with our present invention. Moreover the various individual agents are not impaired with respect to the desirable characteristics which they themselves contribute to the lubricating compositions.

While we have described our invention hereinabove with reference to various preferred forms and embodiments, and with reference to a specific example, it will be understood that our invention is not limited to the details of such illustrative embodiments or example but may be variously practiced and embodied within the scope of the claims hereinafter made. Moreover, while we have in certain instances specifically given certain preferred ranges and proportions, it will be understood that our invention is not limited thereto and that such preferred ranges and proportions are in general selected for particular products and particular purposes; variations in proportions and in the methods of preparation result in products of different characteristics, such products having individual advantages and utilities.

What we claim is:

1. The method of preparing an oil-soluble organic phosphorus compound suitable as an improvement agent for hydrocarbon oils and effective to impart extreme-pressure characteristics to such oils, which comprises reacting an olefin and a phenol in the presence of sulfuric acid and treating at least a portion of the resultant product with phosphorus oxychloride to obtain a final product containing from about one to about five per cent of phosphorus.

2. The method of preparing an oil-soluble organic phosphorus compound suitable as an improvement agent for hydrocarbon oils, which comprises reacting phosphorus oxychloride with a water-insoluble reaction product of a phenol

and an olefin, said product having anti-oxidant properties when added to a hydrocarbon oil, the amount of phosphorus oxychloride being such that substantial but not complete reaction is obtained, thereby incorporating sufficient phosphorus into the final product to give the final product the property of imparting extreme-pressure characteristics to hydrocarbon oil, when added thereto, while retaining to a substantial extent the anti-oxidant value of the aforesaid phenol-olefin reaction product.

3. A method of lubricating bearing surfaces which comprises maintaining between bearing surfaces, one of which is an alloy of the class consisting of binary and ternary alloys of cadmium, silver, nickel, copper and lead, a film of lubricating oil which initially produces an effective lubricating action but which would normally tend to corrode the aforesaid alloy, and maintaining the effectiveness of the lubricating oil by incorporating therein, in a small but sufficient proportion substantially to improve the extreme-pressure characteristics of the oil, a reaction product of phosphorus oxychloride and an alkylated phenol, said alkylated phenol being a phenol-olefin reaction product insoluble in water and in dilute aqueous alkali solution and being a compound selected from the class consisting of secondary and tertiary alkylated phenols, and said first-mentioned reaction product containing not more than about 5 per cent of phosphorus.

4. The method of preparing an oil-soluble organic compound suitable as an improvement agent for highly paraffinic lubricating oils, which comprises reacting an olefin and a phenol in the presence of a catalyst, neutralizing the resultant product, treating a portion of the product with phosphorus oxychloride, treating a second portion with phosphorus pentasulfide, and blending the resultant phosphorus-containing products to obtain a final product soluble in highly paraffinic oil and containing not more than about five per cent of phosphorus.

5. The method of preparing an oil-soluble organic compound suitable as an improvement agent for highly paraffinic lubricating oils, which comprises reacting an olefin and a phenol in the presence of a catalyst, neutralizing the resultant product, treating a portion of the product with phosphorus oxychloride, treating a second portion with phosphorus trichloride, and blending the resultant phosphorus-containing products to obtain a final product soluble in highly paraffinic oil and containing a total of not more than about five per cent of phosphorus.

6. The method of preparing an oil-soluble organic compound suitable as an improvement agent for highly paraffinic oils, which comprises reacting an olefin and a phenol in the presence of a catalyst, neutralizing the resultant product, and treating at least a portion of the neutralized product with a mixture of phosphorus oxychloride and phosphorus trichloride to obtain a final product soluble in highly paraffinic oil and containing not more than about five per cent of phosphorus.

7. An improvement agent for hydrocarbon lubricating oils comprising a reaction product of phosphorus oxychloride and an alkylated phenol, said alkylated phenol being a phenol-olefin reaction product insoluble in water and in dilute aqueous alkali solution and being a compound selected from the class consisting of secondary and tertiary alkylated phenols, and said first-

mentioned reaction product containing not more than about 5 per cent of phosphorus.

8. A motor oil normally tending to produce corrosion of bearing metals of the class consisting of alloys of cadmium, silver, nickel, copper and lead, under conditions of automotive use, having added thereto a small proportion, not more than two per cent, of a reaction product of phosphorus oxychloride and an alkylated phenol, said alkylated phenol being a phenol-olefin reaction

product insoluble in water and in dilute aqueous alkali solution and being a compound selected from the class consisting of secondary and tertiary alkylated phenols, and said first-mentioned reaction product containing not more than about 5 per cent of phosphorus and being present in sufficient amount substantially to retard corrosion.

TROY LEE CANTRELL.  
JAMES OTHO TURNER. 10